

C. W. SHERMAN,  
METHOD OF MAKING CAST METAL CAR WHEELS.  
APPLICATION FILED NOV. 22, 1917.

1,264,338.

Patented Apr. 30, 1918.

2 SHEETS—SHEET 1.



Clifton W. Sherman  
by George P. Popp  
Attorneys.

C. W. SHERMAN,  
METHOD OF MAKING CAST METAL CAR WHEELS,  
APPLICATION FILED NOV. 22, 1917.

1,264,338.

Patented Apr. 30, 1918.

2 SHEETS—SHEET 2.

Fig. 3.



Fig. 4.



Inventor  
Clifton W. Sherman  
by Geyer & Popp  
Attorneys

# UNITED STATES PATENT OFFICE.

CLIFTON W. SHERMAN, OF BUFFALO, NEW YORK.

## METHOD OF MAKING CAST-METAL CAR-WHEELS.

1,264,338.

Specification of Letters Patent. Patented Apr. 30, 1918.

Original application filed November 3, 1914, Serial No. 870,057. Divided and this application filed November 22, 1917. Serial No. 203,310..

*To all whom it may concern:*

Be it known that I, CLIFTON W. SHERMAN, a citizen of the United States, residing at Buffalo, in the county of Erie and State 5 of New York, have invented new and useful Improvements in Methods of Making Cast-Metal Car-Wheels, of which the following is a specification.

This invention relates to an improvement 10 in the method of making cast metal car wheels.

The invention has for its object the production of cast car wheels in which the formation of the different sections is such that 15 the bearing surface of the tread or rim is hard, so as to increase its wearing capacity, the bore of the hub is soft to permit of easily machining the same in order to properly fit the axle; to distribute the metal to the supporting plates and brackets forming the 20 body which are of smaller sectional area than the hub and rim, so as to produce a casting without shrinkage strains, spongy spots or other deformation which would impair 25 the strength of the casting and to eliminate formation strains.

This application is a division of an application filed by myself November 3, 1914, Serial #870,057.

30 In the accompanying drawings:

Figure 1 is a vertical section of a molding flask for producing a car wheel in accordance with my invention, taken on line 1—1, Fig. 2. Fig. 2 is a horizontal section taken 35 on line 2—2, Fig. 1. Fig. 3 is a vertical section of a car wheel embodying my improvements, taken on line 3—3, Fig. 4. Fig. 4 is a bottom plan view thereof.

Similar characters of reference indicate 40 corresponding parts throughout the several views.

In its general construction, the wheel containing my improvements comprises a hub 1, an annular rim or tread 2 arranged concentrically around the hub and provided at 45 its lower edge with a laterally projecting annular flange 3, and a body or supporting member connecting the hub and rim. The upper unflanged edge of the rim is arranged 50 higher or above the upper end of the hub, as shown in Fig. 3. Although the body or supporting member may be variously constructed so far as the details are concerned, that shown in the drawings is suitable and

comprises a horizontal plate or disk which 55 is dished downwardly and connected at the outer edge of its elevated outer part 4 with the upper unflanged edge of the rim while the inner edge of the inner depressed part 5 of said plate is connected with the upper 60 end of the hub, an annular row of outer brackets 6 connecting the underside of the plate with the rim and terminating at their inner ends short of the hub and an annular row of inner brackets 7 connecting the underside of said plate with the hub and terminating at their outer ends short of the rim.

In addition to the inner and outer brackets the plate is preferably provided on its underside with an annular row of intermediate brackets 8 which terminate at their outer and inner ends short of the rim and hub, respectively. The several brackets are interspaced relatively to each other and the inner ends of the outer brackets and the 75 outer ends of the inner brackets overlap each other, while the intermediate brackets overlap the opposing ends of the inner and outer brackets, as shown in Fig. 4. The outer brackets are preferably so constructed 80 that the sectional area of the same gradually increases from the outer ends toward the inner ends thereof, the inner brackets gradually increase in sectional area from their inner ends toward their outer ends, the 85 intermediate brackets gradually increase in sectional area from their outer and inner ends toward the central parts of the same, as shown in Fig. 4, and the plate gradually increases in sectional area from its inner 90 and outer edges to that part thereof intermediate of its inner and outer edges, as shown in Fig. 3.

If desired, the plate may also be provided with an annular strengthening bead 9 which 95 is preferably arranged on the upper side between the hub and rim and formed with the outer brackets, the inner brackets, and the intermediate brackets. Each of the brackets is further preferably provided on its opposite sides adjacent to said bead with swells or ribs, as shown at 6<sup>a</sup>, 7<sup>a</sup>, 8<sup>a</sup>, for a purpose 100 which will presently appear. The various elements of the wheel just described are all formed integrally.

Within the bore of the hub the same is provided with an inner chill, lining or tool piece 10 preferably of tubular form and con-

structed of soft or low carbon steel. This lining is preferably secured to the hub by placing the lining within the mold in which the cast parts of the wheel are formed, so that a fused joint is produced between the hub and lining which knits the same together as effectively as though the same were constructed in one piece of metal. To further secure the hub and lining against longitudinal displacement relatively to each other the periphery of the lining is provided with a plurality of laterally projecting members 11 which are preferably in the form of annular ribs, flanges or collars and which are embedded in the metal of the hub so that the lining is securely anchored against displacement. Ordinarily the pouring of molten metal against or around cold metal, as occurs when pouring metal against the metal hub lining, would produce cracks in the casting owing to the expansion of the cold metal which prevents proper shrinkage of the casting. This difficulty is overcome in the present instance by making the hub lining collapsible or contractible and in the preferred construction of hub lining this is accomplished by making the same of a plurality of sections which are separated from each other by longitudinal joints 10<sup>a</sup>, the space or gap at each of these joints being bridged by a longitudinal flange 11<sup>a</sup> arranged on the longitudinal edge of one lining section and lapping over the opposing longitudinal edge of the adjacent lining section, as shown in Fig. 2.

A wheel of this construction when produced by casting the metal of the hub against the soft steel lining produces a hub the bore of which can be easily machined to fit the axle upon which the same is to be mounted. The bearing surfaces of the rim and flange are also made solid and hardened by pouring the metal forming these parts against a heavy chill. The nature of the metal forming the rim section of the wheel is such as to produce hardness or lend itself to be hardened under proper heat treatment and rapid cooling. Owing to the above described construction of the wheel, the formation of the flanged rim is effected rapidly and uniformly while the pouring of the metal proceeds at a uniform rate into the mold at the hub, and during such pouring, the formation of the flanged rim does not begin until practically the entire hub and the inner parts of the body are formed comprising the depressed inner part of the plate, the inner brackets and the intermediate brackets.

A mold suitable for producing this wheel is shown in Figs. 1 and 2 and as there shown, the same comprises a bottom plate 12, a drag or nowel 13 filled with sand and resting on the bottom plate and forming the lower section of the molding flask, a cope 14 filled

with sand and forming the upper section of the flask, an iron chill or chiller 15 arranged between the drag and cope and forming the intermediate part of the flask, and a core 16 arranged centrally in the flask. The lining 10 is placed in the mold around the core 16, the joints between the lining sections at the upper and lower ends thereof being closed by the adjacent parts of the sand in the flask and the outer longitudinal edges of these joints being closed by a wash of clay or the like. The fluid metal is poured into the cavity formed between the several flask members through a gate or sprue 17 which is formed in the central part of the cope and opens into the upper end of the hub section of the mold cavity.

The outer chill or chiller 15 preferably forms that part of the mold which extends from the back or upper side of the rim flange upwardly across and above the load line 18 of the wheel so that the bearing surface of the flange and the adjacent part of the bearing surface of the rim which receives the wear of the load is densely formed and hardened.

At a suitable number of places the cope of the molding flask may be provided with risers 19 which open into the mold cavity at the heaviest sectional area of the brackets and plate. This heavy sectional area can be located at any suitable point between the rim and the hub, it being the aim to keep this area of metal molten or in a pasty condition until the heavier rim and hub sections have congealed with the assistance of the chillers 10 and 15 and in this way assist in relieving the strain on the lighter plate and bracket sections.

As the molten metal is poured through the sprue into the mold cavity, the same first enters the hub cavity and begins filling the latter from its lower end upwardly. After the lower end of the hub has been formed the continued rise of the metal then begins the formation of the inner brackets and by the time the metal reaches the top of the hub cavity the depressed inner part of the plate and the intermediate brackets have been formed. Up to this time the metal has not yet entered the rim cavity and no part of the rim or its flange and adjacent parts have been formed. As the molten metal surrounds the cold hub lining or chill, the latter becomes heated and tends to expand but owing to the slack joints between the sections of the lining, the latter is contracted by one section thereof sliding circumferentially on another, thereby also compensating for the contraction of the hub when the same cools and hardens, so that no cracks are formed in the hub. When the metal rises to that part of the mold cavity where the central part of the plate cavity joins with the elevated bead cavity and the inner

elevated ends of the outer bracket cavities, the continued inflow of metal through the sprue causes the metal thenceforth to flow rapidly downwardly and outwardly through 5 the outer bracket cavities and fill the rim cavity so that the rim quickly forms with the outer brackets and when the metal reaches the top of the rim the outer elevated part of the plate and the adjacent part 10 of the intermediate brackets have also been filled. In this manner the inner part of the wheel will be formed first followed by the formation of the outer part and the molten metal will rise twice as fast as usual in the 15 mold, particularly in the tread section, with a given speed of pouring. After the mold cavity as a whole has been filled the continued inflow of metal for a brief period through the sprue causes a quantity of the 20 metal to enter the risers and form a surplus or head of molten metal.

The above described quick and uniform formation of the flanged rim section is secured while the molten metal enters the mold 25 cavity at a uniform rate throughout the casting operation.

The metal lying against the rim chill and hub chill shrinks, solidifies and contracts first and the plates and brackets and inner side 30 of rim and outer side of hub sections are properly fed by the head or surplus of reserve molten metal in the risers which flows from the same outwardly through the outer brackets and outer parts of the plate, bead 35 and intermediate brackets to the rim, and inwardly through the inner brackets and inner parts of the plate to the hub, thereby compensating or allowing for any shrinkage and contraction in the metal forming the plate, 40 rim and hub and preventing the formation of any defects which would weaken or affect the strength of the wheel, such as shrinkage holes, spongy spots or piping. The pressure of molten metal tends to strain the congealed 45 circular rim section. This combined with the resistance of the congealed plate section during the cooling period tends to form vertical cracks on the bearing surface of the rim or tread commonly known as chill 50 cracks. The cavity in the mold forming the bead serves as a gate for obtaining a proper distribution of the metal from the heads to all the brackets and all parts of the plate section and the inner part of the rim 55 and the outer part of the hub, and in the finished wheel the bead formed in the bead cavity materially strengthens the wheel. The movement of the metal from the risers to the rim and hub in the manner described is 60 facilitated by the gradual enlargement of the sectional area of the mold cavity from the rim cavity inwardly toward the risers and from the hub cavity outwardly toward the risers, this being secured by enlarging 65 the plate from the hub and rim toward the

risers, as shown in Figs. 1 and 3, enlarging the outer brackets inwardly, enlarging the inner brackets outwardly, enlarging the intermediate brackets from their extremities to the bead which connects the central parts 70 of the last mentioned brackets, as shown in Figs. 2 and 4, and by the cavities forming the swells 6<sup>a</sup>, 7<sup>a</sup> and 8<sup>a</sup> on the brackets, thereby allowing proper contraction of the rim section in its congealed state and avoiding 75 the defective deformation of vertical chill cracks in the face of the tread. This enlargement of the plate brackets also tends to slow up the setting of the metal contained therein which allows the circumferential and radial 80 shrinkage and contraction of the previously congealed tread section to take place without producing defects known as chill cracks.

The objects of this increased sectional area 85 of the plate and bracket are thus attained, one to properly assist in feeding the molten metal to the plate and bracket sections adjacent to the rim, and the other to keep this sectional area molten so that the rim section can properly contract.

The chilling of the tread increases the density of the metal therein as well as the hardness thereof. The chilling of the hub with lighter chiller only increases the density 95 of the metal in the same because in the proper formation the hub should be soft and strong. In the manufacture of a wheel of this kind, a high carbon metal is preferably employed which will produce steel too hard for easy 100 machining. The use of an inner hub lining or chill made of soft steel is therefore desirable in order to facilitate the boring or machining of the hub so that the wheel may be properly fitted on its axle. A secondary object of the chill lining in the hub is to increase the density of metal in the hub, not 105 its hardness, thereby avoiding the use of heavy gates or risers, because it will tend to cool this heavy section of metal quickly and thereby make a uniform and dense casting of 110 the hub.

It will be apparent from the foregoing that a car wheel made in accordance with my invention will be practically free from any defects due to shrinkage strains or other improper formation or conditions which are present in wheels made in accordance with the method heretofore commonly practised.

My improved wheel is therefore much stronger and safer and these advantages are 120 secured in addition to a material decrease in the weight of the wheel and therefore in the cost of the same.

I claim as my invention:

1. The herein-described method of making 125 car wheels consisting in pouring the bearing face of the rim against a chill of metal and pouring the hub against a lining of relatively soft metal.
2. The herein-described method of making 130

car wheels consisting in pouring the bearing face of the rim against a chill of metal and pouring the hub against a lining of relatively soft metal and providing risers in the mold between those portions of the cavity in which the rim and hub are cast.

3. The herein-described method of making car wheels consisting in pouring the bearing face of the rim against a chill of metal and 10 pouring the hub against a lining of relatively soft metal and providing risers in the mold between those portions of the cavity in which the rim and hub are cast and so constructing the mold that its sectional area gradually increases from said rim and hub portions of 15 the cavity toward said risers.

4. The herein-described method of making integral cast metal car wheels having a hub, a rim, a plate connecting the hub and rim 20 and having a depressed inner part and an elevated outer part, inner brackets connecting the depressed part of the plate and the hub, and outer brackets connecting the elevated part of the plate and the rim, consisting 25 in first casting the hub, inner brackets and depressed part of the plate and then casting the outer elevated part of the plate, the outer brackets and the rim during a uniform pouring of the molten metal.

30 5. The herein-described method of making an integral cast metal car wheel which consists in first casting the entire hub and inner part of the supporting body and immediately

thereafter casting the outer part of the supporting body and the rim of the wheel.

35

6. The herein-described method of making integral cast metal car wheels having a hub, a rim, a plate connecting the hub and rim, inner brackets connecting the inner part of the plate and hub and outer brackets connecting the outer part of the plate and the rim, consisting in first casting the hub, inner brackets and inner part of the plate followed immediately thereafter by the casting of the outer brackets, outer part of the plate 40 and the rim.

7. The herein-described method of making cast metal car wheels having a hub, a rim, a plate connecting the hub and rim, inner brackets connecting the inner part of the 45 plate and hub and outer brackets connecting the outer part of the plate and the rim, consisting in first casting the hub, inner brackets and inner part of the plate followed immediately thereafter by the casting of the outer brackets, outer part of the plate and the 50 rim during an uninterrupted and uniform pouring of the metal into the mold.

8. The herein-described method of making integral cast metal car wheels having a hub, 55 a rim, and a supporting body connecting the hub and rim, consisting in first casting the entire hub and inner part of the supporting body and then casting the outer part of the supporting body and the rim.

CLIFTON W. SHERMAN.